

Patented Oct. 15, 1940

2,218,185

# UNITED STATES PATENT OFFICE

2,218,185

## STABILIZERS FOR FIBROUS TEXTILE MATERIALS

William P. ter Horst, Packanack Lake, N. J., assignor to United States Rubber Company, New York, N. Y., a corporation of New Jersey

No Drawing. Application February 1, 1939,  
Serial No. 254,047

### 10 Claims.

(Cl. 21—4)

This invention relates to stabilizers for cotton and other fibrous textile materials whereby to retard their deterioration when exposed to atmospheric influences.

5 According to the invention the textile material is treated with an acidyl-amino diarylamine having the general formula



10 where  $R_1$  represents an aryl group,  $R_2$  an arylene group and  $Y$  an acidyl group and  $n$  is one or two depending on whether  $Y$  is monovalent or di-  
15 valent. Among such materials are m-acetamino-phenyl beta-naphthylamine, m-(p-toluene-sulfonylamino)-phenyl beta-naphthylamine, p-acet-  
20 amino-diphenylamine, p-(p-toluene-sulfonylamino)-diphenylamine, p-(p-toluene-sulfonylamino)-phenyl p-tolylamine.

Particularly effective are para-(para-toluene  
25 sulfonylamino) diphenylamine



and its homologs such as para-(para-toluene  
25 sulfonylamino)-phenyl para-tolylamine



The following tests made on pieces of cotton duck, exposed to the action of sunlight and the  
30 mercury vapor sunlamp, when treated with the present chemicals are shown below. The tensile strength and bursting strength are in pounds per square inch.

Examples of aminodiarylamines the acidyl derivatives of which are included within the scope of the invention are p-amino-diphenylamine; p-amino-phenyl tolylamine, for example, p-amino-phenyl o-tolylamine and p-aminophenyl p-tolylamine; mono-beta-naphthyl-p-phenylene diamine, mono-alpha-naphthyl-p-phenylene diamine, mono-beta-naphthyl-m-phenylene diamine, and mono-alpha-naphthyl-m-phenylene diamine; and examples of acidyl groupings are those from formic acid, 10 acetic acid, butyric acid, stearic acid, benzoic acid, furoic acid, carbonic acid, phthalic acid, succinic acid, maleic acid, malonic acid, benzene sulfonic acid, toluene sulfonic acid, and oxalic acid. 15 Carbonic, phthalic, succinic, maleic, malonic, and oxalic acids are examples wherein the acidyl group is di-valent and is to be combined with two moles of the chosen amino-diarylamine.

The chemicals may be applied in the form of 20 solutions or emulsions, but preferably in solution in some suitable solvent, to all manners of textile goods that usually deteriorate when exposed to sunlight such as sails, tents, awnings, clothing, sports shoe fabric, netting used in agriculture to protect plants, rope, etc.

Having thus described my invention, what I claim and desire to protect by Letters Patent is:

1. A process of stabilizing cellulosic fibrous textile materials against deterioration which 30 comprises treating the same with an acidyl-amino diarylamine.

2. A process of stabilizing cellulosic fibrous textile materials against deterioration which comprises treating the same with an aryl sulfonyl-amino diarylamine. 35

3. A process of stabilizing cellulosic fibrous textile materials against deterioration which comprises treating the same with a toluene-sulfonyl-amino diarylamine. 40

4. A process of stabilizing cellulosic fibrous textile materials against deterioration which comprises treating the same with para-(para-toluene sulfonylamino)-phenyl para-tolylamine. 45

5. A process of stabilizing cellulosic fibrous textile materials against deterioration which comprises treating the same with para-(para-toluene sulfonylamino) diphenylamine. 50

6. Cellulosic fibrous material containing in combination with the fibres thereof an acidyl-amino diarylamine, whereby to stabilize the fibres against deterioration.

7. Cellulosic fibrous material containing in 55 combination with the fibres thereof an aryl sulfonylaminod diarylamine, whereby to stabilize the fibres against deterioration.

8. Cellulosic fibrous material containing in 60 combination with the fibres thereof a toluene-

|                                                                                                                                 | Warp tensile strength | Filling tensile strength | Bursting strength |
|---------------------------------------------------------------------------------------------------------------------------------|-----------------------|--------------------------|-------------------|
| Cotton duck unexposed.....                                                                                                      | 173                   | 138                      | 35                |
| Cotton duck exposed 2 months on roof.....                                                                                       | 125                   | 114                      | 25                |
| 40 Cotton duck treated with 5% solution of para-(toluene sulfonylamino) phenyl-para-tolylamine exposed 2 months on roof.....    | 164                   | 135                      | 31                |
| Cotton duck treated with 2% sol. of para-(toluene sulfonylamino)-phenyl para-tolylamine exposed 2 months on roof.....           | 146                   | 144                      | 30                |
| 45 Cotton duck treated with 1% sol. of para-(toluene sulfonylamino)-phenyl para-tolylamine exposed 2 months on roof.....        | 141                   | 119                      | 29                |
| Cotton duck treated with 5% sol. of para-(toluene sulfonylamino)-diphenylamine, exposed 2 months on roof.....                   | 154                   | 137                      | 30                |
| 50 Cotton duck exposed 3 months on roof.....                                                                                    | 78                    | 79                       | 15                |
| Cotton duck treated with 5% sol. of para-(toluene sulfonylamino)-phenyl para-tolylamine; then exposed 3 months on roof.....     | 90                    | 110                      | 26                |
| 55 Cotton duck exposed under mercury vapor sunlamp during 144 hours.....                                                        | 35                    | 39                       | -----             |
| Cotton duck treated with 5% sol. of para-(toluene sulfonylamino)-diphenylamine, exposed under mercury vapor lamp 144 hours..... | 68                    | 67                       | -----             |

sulfonylamino diarylamine, whereby to stabilize the fibres against deterioration.

9. Cellulosic fibrous material containing in combination with the fibres thereof para-(para-toluene sulfonylamino)- phenyl para-tolylamine, whereby to stabilize the fibres against deterioration.

10. Cellulosic fibrous material containing in combination with the fibres thereof para-(para-toluene sulfonylamino) diphenylamine, whereby to stabilize the fibres against deterioration.

**WILLIAM P. TER HORST.**